

## UNITED STATES PATENT OFFICE

HANS OSBORG, OF FRANKFORT-ON-THE-MAIN, GERMANY

## PROCESS OF TREATING MOLTEN METALS AND ALLOYS WITH COMPOSITIONS CONTAINING LITHIUM AND PRODUCTS RESULTING FROM SUCH TREATMENTS

No Drawing.

Application filed July 12, 1930. Serial No. 467,625.

The present invention relates to a process of treating, purifying and scavenging metals and alloys in their molten state with an active lithium bearing substance and to products resulting from such a process.

Heretofore, it has been proposed to employ pure metallic lithium for the treatment of metallic substances in their molten state. Attempts to utilize this process, particularly on an industrial scale, have been unsatisfactory for a variety of reasons. The more important reasons were the difficulty of handling pure lithium and incorporating it in a molten mass; the second was relatively high loss of lithium due to volatilization and the like; and the third was the relatively high cost of pure lithium. In other words, when lithium or in fact some other metal of the alkali group or alkaline earth group was added to a molten bath of metal these disadvantages were encountered which in many cases not only counter-balanced any advantages but actually overbalanced any advantages. For instance, in the treating of steel or steel alloys, the temperature of the molten bath was such as to cause a quick volatilization of lithium with the consequence that the treatment only partly occurred or that an excessive amount of lithium had to be used in order to obtain the desired results. In the same way, in the treatment of copper and copper alloys, the lithium added to treating the molten mass of copper was quickly volatilized from the molten bath and the remainder produced results which were not uniform nor satisfactory. For instance, the electrical conductivity of copper when treated with lithium metal was sometimes only 90 to 95% and the fracture as well as the specific gravity were inferior to those usually obtained with the conventional casting methods and procedures employed in the copper industry. In short, the results of treatment of molten metals and alloys with lithium metal or other metals of the alkali group or alkaline earth group alone were un-

satisfactory when carried out on an industrial scale. Various suggestions have been made for remedying the short-comings and disadvantages of the pure lithium treatment, but none, as far as I am aware, has been satisfactory and practical in industrial use.

It is an object of the present invention to provide a process of treating metals and alloys in their molten state so as to obtain the benefits resulting from lithium treatments without the disadvantages noted hereinabove.

It is a further object of the invention to provide a simple, economical and thoroughly satisfactory process of treating metals and alloys in their molten state with active lithium alloy of a metal of the alkali group or of the alkaline earth group so as to improve the characteristics thereof.

It is another object of my invention to provide a process of treating molten metals and molten alloys with an active lithium-bearing alloy of a metal of the alkali group or the alkaline earth group which is capable of being carried into commercial practice on an industrial scale in the ferrous and the non-ferrous industries and which is also capable of producing greater effects than provided by the same amount of lithium and the like.

Other objects and advantages of the invention will become apparent from the following description.

Broadly stated, my invention contemplates the treatment of molten metals and alloys with an active lithium-bearing substance in which the lithium is so bonded that the loss thereof through volatilization and the like is materially reduced. At the same time the lithium bearing substance can function actively to effect improvements in the properties and qualities of the metallic substance under treatment. I have found that in carrying my invention into practice, that lithium-bearing alloys containing members of the alkaline or alkaline earth families or of

mixtures of the foregoing alloys can be utilized in the treatment of metals and alloys in their molten state so as to effect improvements in the properties and qualities in the 5 metals or alloys treated.

The following example is given for illustrative purposes and for a better understanding of carrying my invention into practice.

10 *Example*

In the treatment of iron or steel, for instance the molten metal is contained in a suitable crucible such as a graphite crucible or in a bull ladle or in an ingot mold. To the 15 molten mass I add in any appropriate manner, an active lithium alloy, for example, an alloy of lithium and calcium in an amount sufficient to effect improvements in the properties of the iron or steel. In practice, I have 20 found that up to about 2 parts of an alloy of lithium and calcium having about a 50% lithium content are capable of effectively treating about 100 parts of molten steel or steel alloys.

25 The addition of the active lithium-bearing alloy to the molten metal is preferably effected by plunging the selected amount of active lithium bearing alloys into the molten material in a crucible by any appropriate 30 means such as an inverted cup with side openings or ports or the like. By adding the active lithium-bearing alloy to the molten metal in the aforesaid manner, I am able to effect a thorough distribution of the lithium 35 alloy throughout the molten mass and to effect the proper treatment of said metal to improve the properties and qualities thereof.

When iron or steel or copper or nickel or 40 alloys thereof are treated with one of my active lithium-bearing alloys, the molten mass has a better fluidity and consequently, can be cast very much better than heretofore and gives better and denser castings. In ad- 45 dition, the physical properties of the iron or steel or metal or alloy treated are improved. For instance, there is an increased hardness and corrosive resistance of the metal thus treated and the finished product is relatively 50 or practically free from blow holes, oxygen, sulphur and the like. When copper is treated in this manner, it has a better conductivity than when untreated or treated in conventional ways.

55 The lithium thus added as described hereinabove, improves the crystal structure of the steel; combines with gases, such as oxygen and nitrogen, and also with such detrimental substances as sulphur and phosphorus; in- 60 creases the fluidity of the molten steel and produces denser and sounder casting than produced heretofore. In practice, I prefer in some instances to add the lithium alloy in a mass which is surrounded by or coated with 65 iron silicide. By adding the lithium alloy

in this manner, the procedure is facilitated. If it is desired, a lithium-calcium alloy can be silicided and then the silicided lithium alloy used for the treatment of the molten metal or alloy. The coating of a block or the like of a "lithium alkali" alloy with lithium or silicon may be performed in any appropriate manner but I prefer to utilize the procedures described in my co-pending applications, U. S. Ser. No. 466,584, filed on July 8, 1930, and U. S. Ser. No. 480,283, filed on September 6, 1930.

70 Instead of steel or iron in the examples given above, nickel or alloys thereof or copper or alloys thereof can be treated by the addition of the lithium alloy to the molten metallic mass. Sufficient lithium-bearing substance is added to the molten mass to give the latter a lithium content up to about 1.0%.

75 In some instances, I prefer to employ an alloy of lithium with the metal or alloy to be treated. For example, if steel is to be treated, I use an active lithium alloy containing iron. In the same way, if nickel is to be treated, I use a lithium alloy containing nickel. The lithium alloys should preferably have a lithium content of about 50% and should be silicided or reacted with silicon prior to use.

80 The amount of lithium alloy added to the molten metallic mass depends upon a number of variables as one skilled in the art will readily understand. For example, the percentage of lithium in the lithium alloy will 85 determine in part how much of the substance 90 is to be used. Then again the amount of impurities and gases in the molten metal or alloy and the improvement to be given to the metal or alloy will also have to be taken into account in determining the amount of lithium-bearing substance to be used.

95 It will be observed that the present invention provides a process which can be utilized on an industrial scale to produce successful and satisfactory results which are acceptable 100 to those skilled in the art.

105 It will be further observed that the present invention provides a method for the production of improved metals and alloys which not only can be carried out on a laboratory 110 scale but which also can be carried out on an industrial scale.

115 It will also be noted that the present invention provides a process by the use of 120 which the disadvantages inherent in the sole use of lithium alone or other member of the alkali group or the alkaline earth group alone are avoided and unexpected advantages 125 are obtained from the use of lithium alloys of metals of the alkali group or the alkaline earth group. The lithium in alkali alloys contemplated by my invention are exceedingly active and have an activity which could 130 not be predicted from the prior use of lithium

alone or of other metals of the alkali or alkaline earth groups alone.

Although I have herein described specific illustrative examples of my invention which included specific substances, percentages and the like, it is to be observed that the invention is not to be limited thereto but the scope and spirit thereof is to be determined by the appended claims. For instance, when in the specification and claims I use the term "lithium-alkali alloy" it is intended to mean lithium alloy of a metal of the alkali group or alkaline earth group.

In the same way, when the term "alkali" is used, it is intended to refer to and to include sodium, potassium, calcium, strontium, barium and magnesium which are members of the alkali and alkaline earth families and which have atomic weights greater than 20.

It is also to be understood that the term "alkali" covers mixtures of the foregoing elements.

What is claimed is:

1. The process of treating, purifying and scavenging metals and alloys in their molten state to improve the properties thereof which comprises introducing into a bath of a molten metal or alloy, an active "lithium-alkali" alloy in restricted amounts only sufficient to purify, scavenge and improve the said metal or alloy and insufficient to remain in the finished and treated metal or alloy as a dominant compound or constituent thereof.

2. The process of treating, purifying and scavenging metals and alloys in their molten state to improve the properties thereof which comprises introducing into a bath of molten metal or alloy an active "lithium-alkali" alloy in restricted amounts only sufficient to purify, scavenge and improve the said metal or alloy and insufficient to remain in the finished and treated metal or alloy as a dominant compound or constituent thereof by dipping a solid body of an active "lithium-alkali" alloy into the molten mass or metal to be treated and then stirring the thus treated molten mass to effect a thorough distribution of said "lithium-alkali" alloy.

3. The process of treating, purifying and scavenging metals and alloys in their molten state to improve the properties thereof which comprises introducing into a bath of molten metal or alloy an active "lithium-alkali" alloy in restricted amounts only sufficient to purify, scavenge and improve the said metal or alloy and insufficient to remain in the finished and treated metal or alloy as a dominant compound or constituent thereof by adding a briquette containing an active "lithium-alkali" alloy to a molten mass of metal or alloys to be treated and then causing a thorough mixing of said lithium alloy in said molten metal or alloy.

4. The process of treating, purifying and scavenging metals and alloys in their molten

state to improve the properties thereof which comprises adding a lithium-calcium alloy to a molten mass of metal or alloy to be treated in restricted amounts only sufficient to purify, scavenge and improve the said metal or alloy and insufficient to remain in the finished and treated metal or alloy as a dominant compound or constituent thereof and stirring said molten mass to effect a treatment of the various parts of said mass with said lithium-calcium alloy to effect purification, scavenging, and an improvement of the metal or alloy under treatment.

5. The process of treating, purifying and scavenging metals and alloys in their molten state to improve the properties thereof which comprises introducing into a bath of molten metal or alloy a lithium-calcium alloy in restricted amounts only sufficient to purify, scavenge and improve the said metal or alloy and insufficient to remain in the finished and treated metal or alloy as a dominant compound or constituent thereof by dipping a block of lithium-calcium alloy into the lower portion of a molten mass of the metal or alloy to be treated and distributing said lithium-calcium alloy substantially throughout said mass to effect purification, scavenging and an improvement of the metal or alloy under treatment.

6. The process of treating, purifying and scavenging metals and alloys in their molten state to improve the properties thereof which comprises adding a lithium alloy containing an "alkali" metal to a molten mass of metal or alloy to be treated in restricted amounts only sufficient to purify, scavenge and improve the said metal or alloy and insufficient to remain in the finished and treated metal or alloy as a dominant compound or constituent thereof and stirring said molten mass to effect a treatment of the various parts of said mass with said lithium alloy containing an "alkali" metal.

7. The process set forth in claim 6 in which the lithium alloy is a block of "lithium-alkali" alloy which has its exposed surfaces covered with lithium.

8. The process set forth in claim 6 in which the lithium alloy is a block of "lithium-alkali" alloy which has its exposed surfaces covered with a metallic silicide.

9. The process of purifying, scavenging and improving high melting point metals and alloys which comprises introducing into a molten bath of said metals and/or alloys a "lithium-alkali" alloy in restricted amounts only sufficient to purify, scavenge and improve the said metal or alloy and insufficient to remain in the finished and treated metal or alloy as a dominant compound or constituent thereof.

10. The improved product which comprises a high melting point metal or alloy resulting from the purifying and scavenging treatment

thereof in a molten state with a "lithium-alkali" alloy.

11. The improved product which comprises a high melting point metal or alloy resulting from the purifying and scavenging treatment thereof in a molten state with a lithium-calcium alloy.

12. An article of manufacture comprising an improved metal or alloy resulting from the purifying and scavenging treatment thereof in a molten state with a "lithium-alkali" alloy in restricted amounts, only sufficient to purify, scavenge and improve the said metal or alloy and insufficient to remain in the finished and treated metal or alloy as a dominant compound or constituent thereof.

13. An article of manufacture comprising an improved metal or alloy resulting from the purifying and scavenging treatment thereof in a molten state with a lithium-calcium alloy in restricted amounts only sufficient to purify, scavenge and improve the said metal or alloy and insufficient to remain in the finished and treated metal or alloy as a dominant compound or constituent thereof.

14. An article of manufacture comprising an improved metal or alloy containing a trace of "lithium-alkali" alloy, remaining in said metal and alloy from the treatment thereof in a molten state with said "lithium-alkali" alloy in restricted amounts only sufficient to purify, scavenge and improve the said metal or alloy and insufficient to remain in the finished and treated metal or alloy as a dominant compound or constituent thereof.

In testimony whereof I have hereunto set my hand.

HANS OSBORG.

40

45

50

55

60

65